

Aug. 2, 1960

S. S. FIERKE ET AL

2,947,628

MULTILAYER PRINT FILM HAVING INCORPORATED COLORING MATERIAL

Filed Oct. 12, 1956

**Fig. 1**



**Fig. 2**



*Scheuring S. Fierke  
Homer W. J. Cressman*  
INVENTORS

*By*  
*Samuel J. Mayne*

*W. H. M. Jewell*

ATTORNEY & AGENT

1

2,947,628

## MULTILAYER PRINT FILM HAVING INCORPORATED COLORING MATERIAL

Scheuring S. Fierke and Homer W. J. Cressman, Rochester, N.Y., assignors to Eastman Kodak Company, Rochester, N.Y., a corporation of New Jersey

Filed Oct. 12, 1956, Ser. No. 615,546

7 Claims. (Cl. 96—74)

This invention relates to photography and particularly to a multi-layer photographic film having a light filtering material incorporated therein.

In the usual sensitivity arrangement of three-layer photographic film, the red-sensitive emulsion layer is coated adjacent the support and this is followed in order by the green-sensitive emulsion layer and the blue-sensitive emulsion layer. It is customary to form a cyan dye image in the red-sensitive layer, a magenta dye image in the green-sensitive layer and a yellow dye image in the blue-sensitive layer. It is also well known that a different sensitivity arrangement may be used in which either the red sensitive layer or the green sensitive layer is coated outermost for the purpose of improving definition. It is well known that the definition of the resulting color picture is determined to a large extent by the cyan and magenta dye image and that the overall definition can be improved by arranging the three emulsion layers so that the layer containing the cyan or magenta dye image is outermost and the layer containing the yellow dye image is adjacent the support or farthest from the exposing light. This arrangement is described, for example, in Baker U.S. Patent 1,867,301 and Tarbin U.S. Patent 1,871,479.

When this inverted sensitivity order is used, it is frequently necessary to employ a blue-sensitive emulsion layer, that is, the layer adjacent the support, having a higher blue light speed than would be required if the blue-sensitive layer were outermost. Whether for this or other reasons, it has been found that the blue-sensitive emulsion layer tends to scatter any red or green light reaching it after passing through the upper layers and reflect part of it back to the upper layers, and thereby to reduce the overall definition of the resulting picture. This light scattering in the bottom layer of the film is a serious defect in films using this sensitivity arrangement.

It is therefore an object of the present invention to provide a novel means for preventing light-scattering in multilayer films, either of light passing to lower emulsion layers, or of light reflected from lower to upper emulsion layers. A further object is to retain the advantages of coating the green-sensitive or red-sensitive layer outermost in a multi-layer film and at the same time to reduce or overcome the disadvantage of light scatter caused by the blue-sensitive emulsion layer. A further object is to provide a novel multi-layer photographic film.

These objects are accomplished by including in one of the layers such as one or more of the emulsion layers or an organic colloid interlayer, an internal latent image silver halide emulsion to which is adsorbed a non-image forming coloring material such as one or more optical sensitizing dyes for silver halide absorbing up to 100% of the light to which any emulsion layer above the colored layer is sensitive and substantially no light to which an emulsion layer below the colored layer is sensitive, and when present in an emulsion layer, the coloring material absorbing up to 75% of the light to which that emulsion

2

layer is sensitive. In the case of the blue-sensitive lower layer, the dye in that layer might absorb a major amount of visible light to which the green and red-sensitive emulsions are sensitive and a minor amount of blue light. Thus the green and red-sensitive emulsions could contain both green-light-absorbing and red-light-absorbing dyes or only green-light-absorbing or red-light-absorbing coloring materials associated with the internal latent image emulsion component. Also, the emulsion layers each contain color-forming compounds capable of reacting with the oxidation products of primary aromatic amino silver halide developing agents to form dyes and generally the color-forming compound in each emulsion is selected to form dye images of color complementary to the sensitivity of the emulsion layer.

The function of the internal latent image emulsion component of the red-sensitive or green-sensitive emulsion layers or the interlayer is to prevent the wandering of the dyes from grain to grain in the emulsion layer or from emulsion to emulsion. Since the internal latent image emulsions are not developable in the surface developers used in developing the color films described, they do not interfere with the formation of the colored images in the emulsion layers but since the internal latent image emulsions are readily removable from the films in the processing solutions such as the fixing bath, the coloring material is removed from the emulsion layers together with the internal latent image emulsion during the processing steps.

One advantage of the use of the internal latent image emulsions to which the red-absorbing or green-absorbing dyes are adsorbed, resides in the fact that since non-wandering narrow-band absorbing dyes are used, the over-all speed of the emulsions is higher by as much as 0.6 to 0.8 log E than when wider band absorbing and more diffusible coloring materials are used for coloring the emulsion layers.

The accompanying drawing shows in cross-sectional view, two modifications of our invention wherein Fig. 1 shows the support 10, such as a cellulose ester film base, having thereon a blue-sensitive emulsion layer 11, a red-sensitive emulsion layer 12 containing a cyan or red-absorbing dye adsorbed onto internal latent image emulsion and a green-sensitive emulsion layer 13 containing a magenta or green-absorbing dye adsorbed onto an internal latent image emulsion. Fig. 2 shows the support 10 having sensitive emulsion layers 14, 15 and 11 sensitive respectively to red, green and blue light, a colloidal silver filter layer 16, and a layer 17 containing magenta optical sensitizing dye adsorbed on internal latent image silver halide.

The film used according to the preferred embodiment of our invention consists of a suitable support such as cellulose ester, synthetic resin or paper having on one side thereof, suitable subbing layers and a blue-sensitive silver halide emulsion layer coated thereon. This is followed by green-sensitive and red-sensitive silver halide emulsion layers either of which may be outermost, although we prefer to coat the green-sensitive emulsion layer last or outermost. Since the green-sensitive and red-sensitive silver halide emulsions are sensitive to blue or violet light in addition to the regions to which they are optically sensitized, it is necessary to prevent the action of blue or violet light on these layers. This may be accomplished either by using as the bottom layer a blue-sensitive emulsion which has much higher blue speed than the green-sensitive and red-sensitive emulsions and exposing the entire film through a yellow filter which absorbs all blue light to which the upper layers are sensitive but not all blue light to which the bottom layer is sensitive, or by using in the upper layers emulsions consisting principal-

ly of silver chloride which has very little sensitivity in the visible blue light region. The emulsion layers contain couplers incorporated as described in Jelley and Vittum U.S. Patent 2,322,027.

According to the preferred embodiment of our invention, the blue-sensitive layer is a silver bromide or silver chlorobromide emulsion sensitive to visible blue light and containing a coupler capable of forming a yellow dye image. The red-sensitive and green-sensitive emulsions are silver chloride or silver chlorobromide emulsions relatively insensitive to visible blue light and containing, respectively, couplers capable of producing cyan and magenta dye images.

The optical sensitizing dyes for silver halide which are adsorbed onto the internal latent image emulsions have narrow-band absorptions primarily in the green or red spectral regions and are strongly adsorbed to the internal latent image emulsion. For example, readily soluble cyanine dyes containing  $\beta$ -naphthothiazole, 5-phenylbenzotriazole, 5-chlorobenzotriazole, and 5-phenylbenzoxazole nuclei are suitable as well as hemi-cyanines, hemi-oxanols and merocyanines, in particular the partially solubilized merocyanines, examples of which appear hereinafter.

The internal latent image silver halide emulsions to which the coloring materials are adsorbed are well known in the art. The internal latent image emulsions are emulsions which form latent images mostly inside the silver halide grains. An internal latent image emulsion, as described on pages 296 and 297 of Mees' "The Theory of the Photographic Process," 1942, is especially useful in our invention. Most of the internal latent image emulsions are silver bromo-iodide emulsions of high iodide content, preferably containing at least 10%-20% of iodide. Burton's emulsion is an emulsion of this type, having a silver iodide content of approximately 40% of the content of silver halide. It is not absolutely essential, however, for the emulsion to contain silver iodide.

Burton's emulsion described in Wall, "Photographic Emulsions," 1929, pages 52 and 53, is prepared as follows:

## A

Silver nitrate \_\_\_\_\_ grams 100  
Water \_\_\_\_\_ cc. 500  
Amonia—to form clear solution.

## B

Potassium bromide \_\_\_\_\_ grams 80  
Potassium iodide \_\_\_\_\_ do. 50  
Soft gelatin \_\_\_\_\_ do. 30  
Water \_\_\_\_\_ cc. 1000

## C

Dry gelatin \_\_\_\_\_ grams 250

B is heated to 70° C., and A, cold, added to B with constant shaking, digested for 20 minutes at 50° C., and allowed to cool slowly. C is added after being allowed to swell for 20 minutes in water, drained and melted. The emulsion is then set and washed.

An internal latent image emulsion made as described in the Davey and Knott U.S. Patent 2,592,250 is particularly useful in our invention. This emulsion is prepared by first forming in the absence of ammonia and in one or more stages silver salt grains consisting at least partly of a silver salt which is more soluble in water than silver bromide, subsequently converting the grains to silver bromide or silver bromoiodide and if the silver iodide content of the emulsion is less than 6% calculated on the total silver halide, treating such grains with an iodide compound to bring the silver iodide up to at least 6%, ripening preferably in the absence of ammonia and then either washing out some of the soluble salts or washing out the whole of the soluble salts, followed by the addition of soluble salts such as soluble

chloride or bromide. An example of an emulsion made in this way is as follows:

## Solution No. 1:

5 Inert gelatin \_\_\_\_\_ 20 grams  
KCl \_\_\_\_\_ 20 grams } at 40° C.  
Water \_\_\_\_\_ 560 cc.

## Solution No. 2:

10 KCl \_\_\_\_\_ 100 grams } at 45° C.  
Water \_\_\_\_\_ 520 cc.

## Solution No. 3:

AgNO<sub>3</sub> \_\_\_\_\_ 195 grams } at 45° C.  
Water \_\_\_\_\_ 520 cc.

## Solution No. 4:

15 KBr \_\_\_\_\_ 160 grams  
KI \_\_\_\_\_ 40 grams } at 45° C.  
Water \_\_\_\_\_ 500 cc.

Run solutions Nos. 2 and 3 simultaneously into solution 20 No. 1 in a vessel, taking 90 seconds to do this. Then ripen for 1 minute at 45° C. Next add solution No. 4, then ripen for 20 minutes at 45° C. Next add 235 grams of inert gelatin (dry). Then ripen at 45° C. for 15 minutes during which time the gelatin dissolves. Set and shred the emulsion and then wash until free from all 25 soluble bromide and then add about 150 cc. of 10% solution of KCl (by weight), and then add water to make 3½ liters. The tanning developing agents such as described hereinafter may then be added to the melted emulsion.

An internal latent image type of silver halide emulsion 30 may be defined as one which, when a test portion is exposed to a light intensity scale for a fixed time between  $\frac{1}{100}$  and 1 second, and developed for 4 minutes at 20° C. in the ordinary, "surface" developer (Example I), exhibits a maximum density not greater than  $\frac{1}{3}$  the maximum density obtained when the same emulsion is 35 equally exposed and developed for 3 minutes at 20° C. in an internal type developer (Example II). Preferably 40 the maximum density obtained with the surface developer is not greater than  $\frac{1}{10}$  the maximum density obtained when the same emulsion is developed in the internal type developer. Stated conversely, an internal latent 45 image emulsion, when developed in an internal type developer (Example II) exhibits a maximum density at least 5, and preferably at least 10, times the maximum density obtained when the same emulsion is exposed in the same way and developed in a surface developer (Example I).

An ordinary, surface-type developer, that is, one which 50 develops an image only on the surface of the grains of an internal latent image emulsion, is the following:

## Example I

|                                    | Grams |
|------------------------------------|-------|
| p-Hydroxyphenylglycine             | 10    |
| Sodium carbonate (crystals)        | 100   |
| Water to 1 liter.                  |       |
| Development time, 4 min. at 20° C. |       |

An internal type developer, that is, one which develops 55 an image inside the grains of an internal latent image emulsion, is the following:

## Example II

|                                    | Grams |
|------------------------------------|-------|
| Hydroquinone                       | 15    |
| Monomethyl-p-aminophenol sulfate   | 15    |
| Sodium sulfite (anhydrous)         | 50    |
| Potassium bromide                  | 10    |
| Sodium hydroxide                   | 25    |
| Sodium thiosulfate (crystals)      | 20    |
| Water to 1 liter.                  |       |
| Development time, 3 min. at 20° C. |       |

Our invention will now be illustrated by the following examples:

*Example 1.—Red-sensitive emulsion containing red absorber adsorbed to internal latent image emulsion*

To a mixture, preheated to 40° C., of 616.0 g. of an internal latent image emulsion prepared by the method of Davey and Knott above, containing per mole of silver halide 239.0 g. of gelatin in a total weight of 3080.0 g. per mole and 6.0 ml. of a 7½ percent saponin solution was added with stirring a methanol solution (120 ml.) of 60 mg. of 3,3'-dimethyl-9-phenyl-4,5,4',5'-dibenzothiacarbocyanine bromide. The whole was stirred 15 minutes at 40° C. The total weight was 691.0 g.

178 grams of this emulsion containing the red light-absorbing thiacarbocyanine dye were then added to a mixture of the following:

41.0 g. of a cyan dispersion comprising 3.6 g. of 1-hydroxy-2-[-(2,4-diamylphenoxy)-n-butyl] naphthamide, 0.45 g. of 2-hexadecyl-5-methylhydroquinone, 8.1 g. of di-n-butyl phthalate, 24.6 g. of a 10% deashed gelatin solution, and 3.05 ml. of a 5% Alkanol B surfactant solution  
 214 g. of a red-sensitized chlorobromide emulsion (80 percent silver chloride, 20 percent silver bromide) containing 239 grams of gelatin per mole of silver halide in a total weight of 4280 grams per mole  
 0.0895 g. of benzothiazole methiodide in 5.3 ml. of water  
 0.141 g. of mucochloric acid in 5.2 ml. of water  
 15 ml. of 7½% saponin solution  
 Water to a total weight of 525 g.

This red-sensitive emulsion containing a cyan-forming coupler can be cast on a film support provided with a blue-sensitive yellow-forming coupler-containing emulsion layer at a rate of about 17.7 grams per square foot. Over the red-sensitive emulsion layer is coated a green-sensitive emulsion layer containing a magenta-forming coupler and a green light absorbing dye as provided in the following examples. The element can then be exposed in the conventional manner, for example, to a suitable multilayer color negative and dye images developed therein by means of color development. Following removal of the silver images and residual silver halide in the film by bleaching and fixing operations, it is found upon examination of the dye images that the red absorbing dye adsorbed to the internal latent image emulsion component of the red-sensitive emulsion layer has been removed in the processing solutions along with the internal latent image emulsion, and the dye images possessed a high degree of sharpness. The mentioned speed advantages were obtained in this case since the thiacarbocyanine dye was strongly adsorbed to the internal latent image emulsion and the dye had a narrow absorption band with a peak absorption at 680 millimicrons.

*Example 2.—Red-sensitive emulsion containing red absorber adsorbed to internal latent image emulsion*

An internal latent image emulsion 193.0 g. prepared by the method of Davey and Knott above, containing per mole of silver halide 139.0 g. of gelatin in a total weight of 1930.0 g. was treated with 30 mg. of anhydrous-3,3'-di-β-carboxyethyl-5,5'-dichloro-9-ethylthiacarbocyanine hydroxide in 3.0 ml. of a 1% triethylamine solution diluted to a total volume of 30 ml. with methanol. The weight of the sensitized emulsion was 220.0 g.

The final emulsion was then made by mixing the following components:

88 g. of the above internal latent image emulsion containing the thiacarbocyanine red absorber  
 32.8 g. of the cyan dispersion of Example 1  
 55.5 g. of a 10% deashed gelatin solution  
 171.0 g. of the red-sensitive chlorobromide emulsion used in Example 1.

.0071 g. of benzotriazole methiodide in 4.2 ml. of water  
 .0925 g. of mucochloric acid in 3.4 ml. of water  
 10 ml. of 7½% saponin solution  
 Water to total weight of 344.0 g.

This emulsion can be coated at 14.4 g. per square foot and used as described in Example 1 as the red-sensitive emulsion over a blue-sensitive emulsion. When the thiacarbocyanine dye is used as described as a red absorber, spectrophotometric curves showed a narrow-band absorption with a peak at 642 millimicrons.

*Example 3.—Red-sensitive emulsion containing red absorber adsorbed to internal latent image emulsion*

The procedure of Example 2 was repeated except using 15 as a red absorber in the internal latent image emulsion the dye 3,3'-diethyl-5,5'-9-triphenylthiacarbocyanine-p-toluene sulfonate. When the emulsion was employed in a color film as described in Example 1, sharp images were obtained due to the sharp absorption band of the dye having a peak at 626 millimicrons.

*Example 4.—Green-sensitive emulsion containing green absorber adsorbed to internal latent image emulsion*

The internal latent image emulsion (308.0 g.) described 25 under Example 1 was treated in an analogous manner with 20 mg. of 3,3'-triethyl-5,5'-diphenyloxacarbocyanine iodide dissolved in 0.4 ml. of pyridine and 25.0 ml. of acetone. The weight of the sensitized emulsion was 315.0 g.

30 The final emulsion was prepared by mixing the following:

95 g. of the above internal latent image emulsion containing the oxacarbocyanine green absorber  
 39.5 g. of a magenta dispersion containing 2.7 g. of 1-(2,4,6-trichlorophenyl)-3-[3'-2(2',4'-di-tert-amyl phenoxyacetamido)-benzamido]-5-pyrazolone, 0.63 g. of 2,5-diocetylhydroquinone, 6.65 ml. of tri-o-cresyl phosphate, 23.8 g. of a 10% deashed gelatin solution, and 1.97 ml. of a 5% Alkanol B solution  
 40 134.0 g. of a green-sensitized chlorobromide emulsion (80 percent silver chloride, 20 percent silver bromide) containing 239 grams of gelatin per mole of silver halide in a total weight of 4,430 g.  
 45 0.0054 g. of benzotriazole methiodide in 3.2 ml. of water  
 0.0896 g. of mucochloric acid in 3.3 ml. of water  
 10.0 ml. of a 7½% saponin solution  
 Water to a total weight of 330.0 g.

When the emulsion was used as described in Example 50 1 as the green-sensitive emulsion in conjunction with the red-sensitive emulsion of Example 1, a high degree of sharpness was obtained in the dye images and the green and red absorbers were readily removed with the internal latent image emulsions in the fixing bath employed after 55 color development.

*Example 5.—Green-sensitive emulsion containing green absorber adsorbed to internal latent image emulsion*

The green absorber 3,3'-diethyl-4,5,4',5'-dibenzothiacarbocyanine iodide was incorporated into an internal latent image emulsion just as described in Example 2.

The final emulsion was made by mixing the following:

60 66.0 g. of the above emulsion (.03 mole Ag)  
 39.5 g. magenta dispersion described in Example 4  
 134.0 g. of the green sensitive chlorobromide emulsion described in Example 4  
 0.0054 g. of benzotriazole methiodide in 3.2 ml. of water  
 65 0.0734 g. of mucochloric acid in 2.7 ml. of water  
 70 9.0 ml. of a 7½% saponin solution  
 Water to a total weight of 276.0 g.

This emulsion was employed as a green sensitive emulsion in the manner described in Example 1. The image sharpness benefits were derived in part from the narrow

absorption band of the green absorber having a peak absorption at 494 millimicrons.

It will be apparent that the above representative narrow-band red or green absorbers can be incorporated separately or in admixture in the red or green-sensitive emulsions of the color films described. However, as indicated above, it is preferred to incorporate a red absorber in the red-sensitive cyan-forming, coupler-containing emulsion layer overlying the blue-sensitive emulsion layer and thereover a green absorber in a green-sensitive emulsion layer containing magenta-forming coupler.

The multilayer material in which our internal image emulsions having adsorbed optical sensitizing dyes are incorporated may have the sensitive emulsions arranged in any order, that is, with the blue-sensitive emulsion nearest the support or with the green-sensitive or red-sensitive emulsion nearest the support. The internal image emulsion having adsorbed optical sensitizing dye may be in any of these emulsion layers or in an interlayer between emulsion layers, or in an under layer between the support and the emulsion layers, or in a backing layer or over-coating layer. Black and white single-emulsion-layer films may also have the internal image absorbing layer as an overcoat, undercoat or backing layer.

What we claim is:

1. A multilayer photographic element comprising a support having on one side thereof three silver halide emulsion layers separately sensitive to the blue, green and red spectral regions, and each containing non-diffusing color-forming compounds capable of coupling with the oxidation product of a primary aromatic amino silver halide developing agent to form dyes, and in at least one layer on said side of the support an internal latent image silver halide emulsion, the silver halide grains of which are such as to cause a test portion of said latter emulsion upon exposure to a light intensity scale for a fixed time between  $\frac{1}{100}$  and 1 second and development for 3 minutes at 20° C. in the following internal type developer:

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter                 |       |

to give a maximum density at least 5 times the maximum density obtained when the equally exposed silver halide emulsion is developed for 4 minutes at 20° C. in the following surface developer:

|                        | Grams |
|------------------------|-------|
| p-Hydroxyphenylglycine | 10    |
| Sodium carbonate       | 100   |
| Water to 1 liter       |       |

to which emulsion layer is adsorbed a dye absorbing a major amount up to 100% of the light to which any emulsion above the colored layer is sensitive and substantially no light to which an emulsion layer below the dyed emulsion layer is sensitive, and when present in an emulsion layer, the dye adsorbing a major amount up to 75% of the light to which said last-mentioned emulsion layer is sensitive, said blue, green and red-sensitive emulsions being of the ordinary type developable in a surface developer and incapable of development to said density difference under said test conditions.

2. A multilayer photographic element comprising a support having on one side thereof three silver halide emulsion layers separately sensitive to the blue, green and red spectral regions and each containing non-diffusing color-forming compounds capable of coupling with the oxidation product of a primary aromatic amino silver halide developing agent to form dyes, said blue-sensitive emulsion layer being adjacent said support and having

an appreciably higher blue speed than said green-sensitive and red-sensitive emulsions, and in at least one layer on said side of the support an internal latent image silver halide emulsion the silver halide grains of which are such as to cause a test portion of said latter emulsion upon exposure to a light intensity scale for a fixed time between  $\frac{1}{100}$  and 1 second and development for 3 minutes at 20° C. in the following internal type developer:

|                                  | Grams |
|----------------------------------|-------|
| 10 Hydroquinone                  | 15    |
| Monomethyl-p-aminophenol sulfate | 15    |
| Anhydrous sodium sulfite         | 50    |
| Potassium bromide                | 10    |
| Sodium hydroxide                 | 25    |
| 15 Sodium thiosulfate            | 20    |
| Water to 1 liter                 |       |

to give a maximum density at least 5 times the maximum density obtained when the equally exposed silver halide emulsion is developed for 4 minutes at 20° C. in the following surface developer:

|                        | Grams |
|------------------------|-------|
| p-Hydroxyphenylglycine | 10    |
| Sodium carbonate       | 100   |

25 Water to 1 liter to which is adsorbed a dye absorbing a major amount of visible light to which one of said green-sensitive and red-sensitive emulsion layers is sensitive and a minor amount of blue light.

30 3. A multilayer photographic element comprising a support having on one side thereof three integrally united silver halide emulsion layers separately sensitive to the blue, green and red spectral regions and each containing non-diffusing color-forming compounds capable of coupling with the oxidation product of a primary aromatic amino silver halide developing agent to form dyes, said blue-sensitive emulsion layer being adjacent said support and having an appreciably higher blue speed than said green-sensitive and red-sensitive emulsions, and in at least

35 one of said emulsion layers other than the blue-sensitive emulsion layer an internal latent image silver halide emulsion the silver halide grains of which are such as to cause a test portion of said latter emulsion upon exposure to a light intensity scale for a fixed time between  $\frac{1}{100}$  and 1 second and development for 3 minutes at 20° C. in the following internal type developer:

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter                 |       |

55 to give a maximum density at least 5 times the maximum density obtained when the equally exposed silver halide emulsion is developed for 4 minutes at 20° C. in the following surface developer:

|                        | Grams |
|------------------------|-------|
| p-Hydroxyphenylglycine | 10    |
| Sodium carbonate       | 100   |

60 Water to 1 liter to which is adsorbed a dye absorbing a major amount of visible light to which one of said green-sensitive and red-sensitive emulsion layers is sensitive and a minor amount of blue light.

65 4. The photographic element of claim 3 wherein the three emulsion layers on the support are sensitized in order to the blue, red and green spectral regions.

70 5. A multilayer photographic element comprising a support having on one side thereof three integrally united silver halide emulsion layers separately sensitive to the blue, green and red spectral regions and each containing

non-diffusing color-forming compounds capable of coupling with the oxidation product of a primary aromatic amino silver halide developing agent to form dyes, said blue-sensitive emulsion layer being adjacent said support and having an appreciably higher blue speed than said green-sensitive and red-sensitive emulsions, and in said red-sensitive emulsion layer an internal latent image silver halide emulsion the silver halide grains of which are such as to cause a test portion of said latter emulsion upon exposure to a light intensity scale for a fixed time between  $\frac{1}{100}$  and 1 second and development for 3 minutes at 20° C. in the following internal type developer:

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter                 |       |

to give a maximum density at least 5 times the maximum density obtained when the equally exposed silver halide emulsion is developed for 4 minutes at 20° C. in the following surface developer:

|                        | Grams |
|------------------------|-------|
| p-Hydroxyphenylglycine | 10    |
| Sodium carbonate       | 100   |
| Water to 1 liter       |       |

to which is adsorbed a dye absorbing a major amount of red light, and in said green-sensitive emulsion layer said internal latent image silver halide emulsion to which is adsorbed a dye absorbing a major amount of green light.

6. The photographic element of claim 5 wherein the red-sensitive layer is superposed over the blue-sensitive emulsion layer and the green-sensitive emulsion layer is outermost.

7. A multilayer photographic element comprising a support having on one side thereof three integrally united silver halide emulsion layers separately sensitive to the blue, green and red spectral regions and each containing

non-diffusing color-forming compounds capable of coupling with the oxidation product of a primary aromatic amino silver halide developing agent to form dyes, said blue-sensitive emulsion layer being adjacent said support and having an appreciably higher blue speed than said green-sensitive and red-sensitive emulsions, and in an interlayer between said blue-sensitive emulsion layer and the outermost emulsion layer an internal latent image silver halide emulsion the silver halide grains of which are such as to cause a test portion of said latter emulsion upon exposure to a light intensity scale for a fixed time between  $\frac{1}{100}$  and 1 second and development for 3 minutes at 20° C. in the following internal type developer:

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter                 |       |

to give a maximum density at least 5 times the maximum density obtained when the equally exposed silver halide emulsion is developed for 4 minutes at 20° C. in the following surface developer:

|                        | Grams |
|------------------------|-------|
| p-Hydroxyphenylglycine | 10    |
| Sodium carbonate       | 100   |
| Water to 1 liter       |       |

to which is adsorbed a dye absorbing a major amount of visible light to which one of said green and red-sensitive emulsion layers is sensitive and a minor amount of blue light.

#### References Cited in the file of this patent

##### UNITED STATES PATENTS

|           |              |                |
|-----------|--------------|----------------|
| 1,879,806 | Kelley       | Sept. 27, 1932 |
| 2,456,954 | Knott et al. | Dec. 21, 1948  |
| 2,456,956 | Knott et al. | Dec. 21, 1948  |